

A. A. LOCKWOOD,  
SEPARATION OF ORES.  
APPLICATION FILED, NOV. 24, 1917.

1,329,127.

Patented Jan. 27, 1920.

*Fig. 1.*



*Fig. 2.*



*Fig. 3.*



*Fig. 4.*



Witness

Chas. L. Griesemer

Inventor

ALFRED A. LOCKWOOD

By

*W. M. Wetherell*

Attorney

# UNITED STATES PATENT OFFICE.

ALFRED ARTHUR LOCKWOOD, OF MERTON PARK, ENGLAND.

## SEPARATION OF ORES.

1,329,127.

Specification of Letters Patent. Patented Jan. 27, 1920.

Application filed November 24, 1917. Serial No. 203,824.

To all whom it may concern:

Be it known that I, ALFRED ARTHUR LOCKWOOD, a subject of the King of Great Britain and Ireland, and a resident of Merton Park, 5 county of Surrey, England, have invented a certain new and useful Improvement in the Separation of Ores, of which the following is a specification.

My invention has for its object certain 10 improvements in and relating to the separation of sulfid, oxid, carbonate and other ores, as hereinafter described and pointed out in the appended claims.

Certain forms of apparatus may be utilized 15 in the performance of the present process, and by way of illustration reference may be had to the accompanying drawing; in which:—

Figure 1 is a perspective view of a shaking 20 table of the Wilfley type.

Fig. 2 is a detail sectional view showing how the ores suspended in water may be conducted through or between cathode or 25 anode surfaces before being deposited on the shaking table.

Fig. 3 is a detail sectional view showing the riffles of the table shown in Fig. 1 coated with lead or other suitable material.

Fig. 4 is a view similar to Fig. 3 showing 30 the riffles made entirely of lead or other suitable material.

Similar reference characters designate 35 corresponding parts throughout the several figures of the drawings.

It will of course be understood that the 40 details of the apparatus shown in the drawings are simply for the purposes of illustration and the carrying out of my process is not limited to the precise details and arrangement shown.

In carrying out the invention, ores whose metalliferous particles are capable of conducting electricity, are passed either through, over, or between cathode and anode surfaces 45 arranged in close proximity to one another in such manner that said metalliferous particles themselves become temporary cathodes and anodes or vice versa. This causes the deposition of hydrogen or oxygen or both upon such temporary cathodes and anodes, or vice versa, rendering them buoyant and easily separable by flotation and gravitation methods.

In the event of the metalliferous particles 50 being bad or insufficient conductors for gas

deposition, for instance, say, when oxidized particles or carbonates of the metal are being heated, said metalliferous particles are subjected to a preliminary treatment, consisting of agitation in water with a non-miscible substance, such as oil, or the like previously mixed with a finely ground readily conducting material, such as ground graphite, copper pyrites, or galena, with the result that gas emanations will be 60 evolved upon the coated surface as readily as though the whole particle were of a conducting material.

To facilitate the conductivity of the water and to economize the electric power necessary 65 for carrying out the process, a small percentage of a salt of an acid or of an alkali nature may be added as is usual in such cases.

A salient feature characteristic of my invention is that the process is conducted in conjunction with the gravity method using a shaking table of the Wilfley type, but with riffles of a conducting material instead of the ordinary wooden riffles, said conducting 75 riffles being connected up alternately as positive and negative and charged with direct current, so that the lighter metalliferous particles as they travel over said riffles become alternately buoyed with cathode and 80 anode gases.

By reference to the accompanying drawings it will be observed that a form of apparatus for carrying out the foregoing steps is shown. Fig. 1 shows a table T mounted 90 upon a plurality of flexible struts or legs d, and having connected therewith a rod or shaft c which is provided at one end with means for being eccentrically mounted as at e on a shaft f, to which power may be applied by the pulley g or the like. The top surface of this table is provided with a plurality of riffles or ridges r which may be either wood riffles coated with lead or other suitable material as shown in Fig. 3, or solid 95 lead or like material as shown in Fig. 4. In each case, however, the adjacent riffles are charged with a positive and negative current, whereby they become anodes and cathodes for carrying out the electrolytic 100 action used in the present process.

In this manner are the two processes simultaneously carried out, the heavier non-gassed mineral particles being caught, as usual, while the buoyed and gassed mineral 110

particles flow off at the slime end and become entrapped by the usual baffles, the slime being allowed to escape.

It is obvious that the electrification may 5 be performed separately, or on a deck on the gravity table and provided with electrified riffles as above set forth, or two horizontal plates *a* and *b* of conductive material as shown in Fig. 2, close to and above one 10 another may be provided on the gravity table and charged as cathode and anode surfaces, contact being maintained by keeping the intervening space, between the conduct- ing plates, full of water and pulp.

15 This method possesses the advantage that the gas emanations are compressed and work, more or less, under light pressure, enhancing their tendency to attach them- selves to the metalliferous particles.

20 In the event of a plurality of minerals in an ore, these are separated from one an- other as well as from the gangue. For in- stance, with an ore containing blende, ga- lena, and Cu pyrites of different electric 25 susceptibilities, it is found that by suitably manipulating the strength of the electric current, galena and Cu pyrites are extracted together by flotation and the blende from the gangue by gravitation all in one com- 30 bined operation, and by a separate gravity treatment to separate the Cu pyrites from the galena.

When, however, the metalliferous parti- 35 cles are of equal electric conductivity or non-conductivity (as in the case of oxydized ores) a coating, by agitating the ore with electrolytic conducting material such as ground graphite, etc., as previously de- scribed, and an oily liquid has to be resorted 40 to for the selection of the desired mineral, when they are then passed over the electri- fied gravity table as hereinbefore described.

In connection with the feature of the 45 invention which provides for preparing the relatively heavy particles of ore in such a manner that they may be readily separated by the present process, through the use of an oily liquid, it will be understood that any suitable oily liquid may be used such 50 as petroleum residuum or fatty acids, and while it is true that these oils are highly non-conductive, nevertheless, when they are charged to the consistency of paint with finely ground particles of conducting ma- 55 terial, above set forth, and caused to be ap- plied to the particles of ore in a thin film, they readily conduct even weak currents owing to the fact that the finely ground par- ticles contact with each other and form in 60 effect an enveloping film of electrolytic con- ductive material, the oil being merely used as a vehicle for carrying the finely ground conducting substance so as to cause the sur-

face portions or exterior of the extractable mineral particles to be coated by the elec- 65 trolytic conducting material.

Having now described my invention, what I claim as new and desire to secure by Let- ters Patent of the United States is:—

1. A process for separating ore tailings, 70 concentrates and the like consisting in flow- ing a sheet of pulp containing material to be separated over a supporting surface, agi- tating and baffling the pulp during its pas- sage over said surface and passing electric 75 currents through the pulp between baffling elements and thereby evolving gas which ad-heres to and buoys certain of the compo- nents of the pulp relatively to other com- ponents, and collecting the components so 80 buoyed.

2. A process for separating ores which consists in passing finely ground particles of the ore with water into the zone of action of the opposite poles of an electric circuit 85 and simultaneously agitating said water containing the ore together with a non- miscible substance containing a conducting material, whereby the finer particles of ore floating near the top of the water will first 90 be coated with a gaseous envelop by the electric action and be rendered buoyant, while the heavier and poorly conducting parts of the ores which fall by gravity will be coated with the non-miscible conductor- 95 bearing substance, whereby they will also ultimately be surrounded by a gaseous en- envelop and become buoyant.

3. A process for separating ores which consists in adding to the ore in the presence 100 of water an electric conducting substance and an adhesive non-miscible conductor- carrying substance such as an oily liquid, then agitating the whole and subjecting the same to the action of closely adjusted op- posite poles of an electric circuit, whereby 105 the electrolytic action thus produced will cause the ore particles to be surrounded by a gaseous envelop and rendered buoyant.

4. A process for separating ores which 110 consists in separating the mineral particles from the gangue by passing the same with water into the zone of action of opposite poles of an electrical circuit and simulta- neously agitating the water and a non-mis- 115 cible conductor bearing substance which ad-heres to some of the ore particles in prefer- ence to other particles, whereby the metal- liferous particles of ore will be enveloped by a gaseous coating due to the electrolytic 120 action and be rendered buoyant.

In testimony whereof I have affixed by signature hereto this sixth day of Novem- ber, 1917.

ALFRED ARTHUR LOCKWOOD.